

May 21, 1940.

D. J. SULLIVAN

2,201,931

ARTICLE OF MANUFACTURE

Filed Dec. 31, 1937

*Fig. 1*



*Fig. 2*



*Fig. 3*



David J. Sullivan

INVENTOR

BY

*Paul J. Seltz*  
ATTORNEY

## UNITED STATES PATENT OFFICE

2,201,931

## ARTICLE OF MANUFACTURE

David J. Sullivan, Fairfield, Conn., assignor to  
 E. I. du Pont de Nemours & Company, Wil-  
 mington, Del., a corporation of Delaware

Application December 31, 1937, Serial No. 182,725

7 Claims. (Cl. 91—68)

This invention relates to artificial leather, and more particularly, to an improved leather substitute comprising a flexible backing to which is applied an improved coating composition of 5 rubber or rubber-like materials.

Heretofore artificial leathers have been characterized by a lack of leathery feel, despite the numerous expedients that have been employed to make them simulate genuine leather. These 10 artificial leathers heretofore known have all fallen short, to a greater or less degree, of an entirely satisfactory substitute for leather due to a lack of some essential quality of leather. Either they did not look like leather or they 15 were stiff and boardy, or rubbery, or were lacking in draping properties, et cetera.

It was known that rubber coating compounds useful for making leather substitutes could not be embossed with sufficient sharpness and permanency to survive a vulcanizing treatment, unless the coating material contained less than about 50% of rubber and a considerable percentage of earthy fillers such as clay, magnesium carbonate, and whiting. Sometimes fibrous materials were included with more or less earthy 25 filler. These constituents were present in addition to the necessary vulcanizing ingredients, such as zinc oxide together with sulphur, and other desired ingredients, such as coloring, softening, activating and accelerating agents.

However, the leather substitutes made with all such coating compositions failed to approach closely the appearance or character of leather in some important noticeable respect. For example, the substitutes which contained earthy 35 fillers were noticeably unlike leather in that the specific gravity was too high. If they did not actually look like rubber compounds, the material was relatively too heavy for its thickness to be a good substitute for leather, and its feel suggested ordinary oil cloth. Some of the leather substitutes were too boardy and some were too rubbery to resemble leather closely. Many of the 40 materials of the prior art showed edge cracking. Leather substitutes containing light non-earthly and non-fibrous fillers were unlike leather in that they lacked the proper fibrous character of 45 leather and they had in addition some of the defects heretofore noted.

This invention had for an object the preparation of an improved and a more leather-like 50 leather substitute. Other objects were the provision of a rubber coated fabric leather substitute having a leather feel, containing a high 55 content of rubber, having good graining charac-

teristics, which retains embossing marks to a satisfactory degree, which contains an appreciable quantity of newsprint paper or wood fiber in equivalent form, which resembles leather in point of bulk (or specific gravity), which eliminates the "boardy" feel of ordinary leather substitutes, which eliminates the rubbery feel of common substitutes for leather, which is improved with respect to "edge cracking," which has an improved leather-like feel, and which 10 looks like leather. A further object was to provide an artificial leather for garments, gloves, upholstery, and the like, which more closely imitates genuine horse hide or cow hide in appearance and feel than the leather substitutes here- 15 tofore produced. Another object of the invention was the preparation of a rubber containing leather substitute composition which when disposed on a suitable fabric would give a product resembling leather in such characteristics as 20 bulk, feel, appearance and resistance to cracking upon flexing. A general advance in the art and other objects which will appear hereinafter are also contemplated.

It has now been found that a leather-like 25 leather substitute may be produced by applying to a flexible backing either with or without an intermediate rubber cement layer a rubber composition containing an appreciable quantity of wood fiber in the form of newsprint paper evenly 30 dispersed throughout its mass and thereafter vulcanizing the product, coupled if desired, with further finishing treatment or treatments.

From the following description and specific examples in which are disclosed certain embodiments of the invention as well as details of what is believed to be the best mode for carrying out the invention, it will be apparent how the foregoing objects and related ends are accomplished. The quantities are given in parts by 35 weight throughout the application. The written description is amplified by the accompanying drawing in which:

Figure 1 is a sectional view representing somewhat diagrammatically a preferred form of the 45 artificial leather of the invention;

Figure 2 illustrates a product similar to that of Figure 1 in which the top surface finishing coating has been omitted; and

Figure 3 illustrates a product similar to that 50 of Figure 1 in which an additional top surface finishing coating has been applied.

Similar characters refer to similar parts throughout the drawing and specification.

In one embodiment of the invention a web of 55

sheeting indicated by the numeral 1 in Figure 1, weighing 5 ounces per square yard and having one side napped, was dyed black and coated on the unnaped side with a rubber cement composition at the rate of one to two ounces per square yard. This layer in position on the sheeting is designated by the numeral 2 in Figure 1. The composition was spread on the web in the conventional manner. In commercial practice it is applied in one or more spread coats, depending upon the convenience of the operator. Any desired consistency may be obtained by the addition of gasoline. Obviously, more coats of a cement, which has been cut very thin with a solvent like gasoline, are necessary to secure a particular coating than are required with the thicker compositions.

A typical rubber cement composition is given in Example I.

| 30                                                              | Example I | Per cent |
|-----------------------------------------------------------------|-----------|----------|
| Plantation rubber                                               | 40        |          |
| Palm oil                                                        | 1         |          |
| Zinc oxide                                                      | 4         |          |
| 25 Barytes                                                      | 25        |          |
| Whiting                                                         | 28        |          |
| Albasan (antioxidant)                                           | 0.5       |          |
| Trimene base, (triethyl, trimethylene, tri-amine) (accelerator) | 1.0       |          |
| 30 Sulphur                                                      | 0.5       |          |
|                                                                 | 100.0     |          |

After the volatile solvent had been removed 25 from the rubber cement layer 2, a coating 3 of a rubber coating composition was applied to the web over the rubber cement composition at approximately the rate of 14 ounces per square yard. Compositions of this character are preferably 40 applied by a calender. The color of the final product (artificial leather) of this invention is largely determined by the color of the layer 3. A typical example of a rubber coating composition adapted to give black artificial leather is as 45 follows:

Example II

| 50                                                              | Per cent |
|-----------------------------------------------------------------|----------|
| Plantation crepe                                                | 66.635   |
| Palm oil                                                        | 1.000    |
| Carbon black                                                    | 3.500    |
| Zinc oxide                                                      | 4.000    |
| Newsprint paper                                                 | 21.69    |
| "Neozone D" (phenyl beta naphthyl-amine) (antioxidant)          | .75      |
| 55 Trimene base (triethyl trimethylene tri-amine) (accelerator) | 1.75     |
| Sulphur                                                         | .675     |
|                                                                 | 100.000  |

60 A typical specific example of a rubber coating composition for a brown artificial leather is as follows:

Example III

| 65                 | Per cent |
|--------------------|----------|
| Plantation rubber  | 66.00    |
| Iron oxide         | 4.00     |
| Carbon black       | 1.3      |
| Zinc oxide         | 4.00     |
| 70 Newsprint paper | 21.55    |
| "Neozone D"        | .75      |
| Trimene base       | 1.75     |
| Sulphur            | .65      |
|                    | 100.00   |

A typical example of a formula for a green artificial leather is as follows:

Example IV

|                   | Per cent | 5  |
|-------------------|----------|----|
| Plantation rubber | 67.5     |    |
| Green lake        | 2.0      |    |
| Zinc oxide        | 4.0      |    |
| Newsprint paper   | 23.33    |    |
| "Neozone D"       | .75      | 10 |
| Trimene base      | 1.75     |    |
| Sulphur           | .67      |    |
|                   | 100.00   |    |

15 A thin coat 4 of quick drying shellac varnish (comprising shellac dissolved in a mixture of water, denatured ethyl alcohol, ammonia, and soap) was applied to the rubberized surface of the web as it came from the calender. This shellac varnish not only served as a surface finishing coat but also removed the surface tack on the rubberized face of the web so that the same could be rolled up without sticking. In commercial scale manufacture a lint-free liner is run in the roll of web to protect the surface of the 25 unvulcanized rubber coating.

20 The coated web was thereafter passed through embossing rolls (embossing presses have also been used satisfactorily) to give the coating a characteristic leather grain. The assemblage was then 30 vulcanized in a hot air vulcanizing chamber for one and one-half hours at 250° F. (157° C.).

After the vulcanization step the coated surface of the product was treated with a 4% solution of bromine (by volume) in carbon tetrachloride to 35 indurate the shellac varnish layer. The product was thereafter and finally exposed to an atmosphere of ammonia to neutralize the indurated surface.

Wide variations may be made in the rubber 40 coating composition as will be apparent from the above examples. The same is true of the flexible backing and the rubber cement used to coat the same.

Instead of sheeting, any flexible backing can 45 be used, including woven or unwoven fabrics, felt and paper. Special mention may also be made of paper impregnated with rubber or other impregnating media. The back side as well as the front side of the backing may or may not be napped, 50 and in any case may be given a coat of cement to mat the fibers to a certain extent to give the back side of the product a resemblance to the back side of split leather.

55 The invention is not limited to the use of natural rubber. In another embodiment of the invention an unnaped web of sheeting weighing 6 ounces per square yard was coated on one side with a plurality of coats of neoprene cement so that one to two ounces of solids per square yard 60 remained deposited after the solvent had been volatilized by heating. The specific cement used had the following composition:

Example V

| 65                         | Parts |
|----------------------------|-------|
| Neoprene                   | 40    |
| Zinc oxide                 | 4     |
| Extra light calc. magnesia | 4     |
| Sulphur                    | 2     |
| FF wood rosin              | 2     |
| Cottonseed oil             | 2     |
| Whiting                    | 48    |

75 This composition was cut in xylene to the desired consistency before spreading. The preferred 75

coating range is from 3 to 8 ounces (before solvent removal) per square yard.

The xylene having been removed, a neoprene coating composition was applied over the cement layer to the extent of 13 ounces per square yard. This neoprene coating composition was adapted to give a black artificial leather, and had the following specific formula:

| 10 | Example VI                    | Parts |
|----|-------------------------------|-------|
|    | Neoprene                      | 60    |
| 15 | Zinc oxide                    | 6     |
|    | Extra light calcined magnesia | 6     |
| 16 | Sulphur                       | ½     |
|    | FF wood rosin                 | 3     |
| 16 | Newsprint paper               | 20    |
|    | Cottonseed oil                | 3     |

The neoprene coating composition was applied to the fabric web by calendering, and a thin coat of the shellac varnish described above was applied as the product left the rolls. The sheet material was wound up with a lint-free liner and temporarily stored. Thereafter, it was unrolled and passed through an embossing press to give the coated layer a characteristic leather grain. The whole was then subjected to a temperature of 260° F. (162° C.) for three hours in a hot air vulcanizing chamber in order to cure the same.

The surface was then further finished by applying another thin coat of the shellac composition disclosed above.

Neoprene is a plastic polymer of chloroprene and may be prepared by polymerizing chloroprene according to United States Patent 1,950,436 issued March 13, 1934 to Williams. Chloroprene is chloro-2-butadiene-1:3, a liquid whose preparation is described by Carothers, Williams, Collins and Kirby in the Journal of the American Chemical Society, volume 53, page 4203 (1931). The compounding of chloroprene plastic polymer in various manners is understood by those skilled in the art of compounding rubber. Specific technique is described in the "Duprene" Manual issued August 21, 1934, by E. I. du Pont de Nemours and Company of Wilmington, Delaware, and in an article by Bridgewater & Krisman in the Journal of Industrial and Engineering Chemistry, volume 25, page 280 (1932).

The leather substitute from neoprene possesses better resistance to oil and to petroleum products than does the natural rubber product.

The use of other synthetic rubber-like substances such as "Buna," "Thiokol," and the like are not excluded from the present invention. The specific compositions employing such materials vary with respect to the particular demands of the rubber-like substances being employed, as will be well understood by those skilled in the art of compounding rubber and related materials. In each case, however, an amount of newsprint paper equal to from 20% to 50% of the rubber-like material employed is included in the composition, and earthy fillers such as clay, whiting, and barytes are entirely omitted except insofar as they may be required by the characteristics or demands of the particular rubber-like substance being utilized.

It is preferred to use unprinted newsprint paper as the source of the wood fiber in the coating composition, although other similar fibers can be used. In compounding the coating composition it is preferred to tear ordinary unprinted newspaper into sheets of convenient size and add them to the other ingredients of the composition and

then mix and macerate them thoroughly on the mixing roll. The tearing, maceration and shearing action during the mixing process serves to disintegrate the paper thoroughly, and uniformly disperse the resulting fibers throughout the composition. The compositions which are made by the use of newsprint paper have the earlier described properties which give products resembling leather more closely than known leather substitutes. At present there is no known theory which explains the reasons for the superiority or difference.

The preferred results have been obtained by using fibers at least one millimeter long, and preferably fibers whose lengths fall within the range of one to two millimeters, are employed. Newsprint paper carrying fibers of these lengths has been found especially suitable. It seems necessary to use fibers of the aforementioned length in order to produce the best results. Difficulty has been experienced in obtaining good mixing uniformity with fibers longer than about two millimeters. When fibers shorter than about one millimeter are employed the resulting leather substitute has characteristics which approach the unleather-like characteristics of leather substitutes, prepared from the usual earthy fillers.

It is essential that an appreciable quantity of newsprint or equivalent fiber be included in the composition to obtain the desired leather-like effect. It is preferred that the proportion of fiber be about one part to three parts of crude rubber, although any proportion which will allow good embossing characteristics of a rubber compound containing about 50% to about 75% of crude rubber, is within the scope of the invention. When the proportion of fiber is greater than one part to two parts of rubber, it is difficult to disperse the fibers evenly throughout the composition, and the finished leather substitute product has a tendency to become "boardy." When the proportion of fiber is less than one part to five parts of crude rubber, the finished product may feel too rubbery.

The primary object of the rubber or equivalent cement layer is to enable the subsequently applied coating composition containing the fibers to be secured to the backing. It will be apparent, therefore, that if the rubber composition and the backing are of such character that a layer of the coating composition will adhere securely to the backing without the use of a cement layer, the said cement coat can be omitted. Any rubber or rubber-like cement composition may be used for this purpose, said composition including for instance rubber, sulfur, and the usual softeners, fillers, pigments, accelerators, antioxidants, etc.

The softeners, pigments, vulcanizing agents, accelerators, antioxidants, and other usual ingredients in the rubber or rubber-like coating compositions may be varied considerably, both in character and in quantity, as is well understood in the art of compounding rubber.

After application of the coating composition, for example rubber, thin layer of shellac varnish is preferably applied. This varnish may comprise shellac dissolved in ethyl or methyl alcohol or equivalent solvent media and may, if desired, include small amounts of water, soap, ammonia, or other ingredients of shellac varnishes, as will be understood by those skilled in the art. It is not absolutely necessary that a shellac varnish be applied to the rubber or rubber-like coat-

ing on the base, and such a modification is illustrated in Figure 2. After the base has had the rubber or rubber-like coating composition applied, it may be vulcanized and, if desired, subsequently indurated whether or not the shellac coating has been applied. Although it is preferred to subject the product to a halogenizing treatment, this is not necessary as the product may be finished with or without a shellac varnish top layer (as above indicated) and with no halogenizing treatment, or may be finished with a shellac varnished top layer that has not been halogenized.

It will be understood that various decorative surface effects may be produced on the coated web by combinations of embossing and souping, printing, stenciling, etc., as will occur to those skilled in the art. Likewise, varnishing or lacquering of the material over the first shellac varnish layer may be employed to produce a product resembling glazed leather. Such a modification is illustrated in Figure 3, wherein 4 represents the shellac layer and 5 a decorative varnish layer superimposed thereon.

23 The indurating step is not limited to treatment of the artificial leather with bromine dissolved in carbon tetrachloride, as any halogenizing treatment will produce more or less desirable results. For example, the rubber coated web, 20 whether shellacked or not, may be treated with a solution of sulfur chloride or sulfur bromide in carbon tetrachloride, or other halogenizing agents.

The vulcanizing temperature and duration may be widely varied, as will be fully understood by those skilled in the art of coating with rubber compositions.

Although it is preferred to apply the rubber coating composition by calendering, the composition may be thinned by a solvent such as gasoline and applied by spreading repeated coats of the same on the base.

The artificial leather produced in accordance with this invention very closely resembles genuine dressed leather in appearance, feel, pliability, wear, durability and draping qualities, and is superior to artificial leather now on the market in these properties. A particular advantage of this artificial leather, due to the newsprint wood fiber in the rubber coating composition, is its resistance to abrasion and edge cracking at seams and folds, which resistance artificial leather heretofore known does not possess to anything like the same degree.

55 The artificial leather of the present invention is particularly adapted, due to the above mentioned properties, for making garments such as imitation leather coats, leggings, gloves, and belts, and also for making upholstery, quarter-linings, shoes, purses, luggage, etc.

This application is a continuation-in-part of my application Serial No. 53,242 filed December 6, 1935, which was a continuation-in-part of my application Serial No. 513,610 filed February 15, 65 1931.

As many apparently widely different embodiments of this invention may be made without departing from the spirit and scope thereof, it is to be understood that I do not limit myself to the specific embodiments thereof except as defined in the appended claims.

I claim:

1. Process which comprises coating the unnaped side of a sheeting weighing 5 ounces per

square yard dyed black and having one side napped with a rubber cement of the formula

|                                                                | Per cent |
|----------------------------------------------------------------|----------|
| Plantation rubber                                              | 40       |
| Palm oil                                                       | 1        |
| Zinc oxide                                                     | 4        |
| Barytes                                                        | 25       |
| Whiting                                                        | 28       |
| Albasan (anti-oxidant)                                         | 0.4      |
| Trimene base (triethyl, trimethylene, tri-amine) (accelerator) | 1.0      |
| Sulphur                                                        | 0.5      |

until 1 to 2 ounces of cement per square yard have been deposited, applying over the said rubber cement coating a layer of a rubber composition having the formula

|                                                              | Per cent |
|--------------------------------------------------------------|----------|
| Plantation crepe                                             | 66.635   |
| Palm oil                                                     | 1.000    |
| Carbon black                                                 | 3.500    |
| Zinc oxide                                                   | 4.000    |
| Newsprint paper                                              | 21.69    |
| "Neozone D" (phenyl beta naphthylamine) (antioxidant)        | .75      |
| Trimene base (triethyl trimethylene tri-amine) (accelerator) | 1.75     |
| Sulphur                                                      | .675     |

coating the said rubber composition with a thin coat of quick drying shellac varnish, embossing the resulting laminated sheet material, vulcanizing the said embossed material, indurating the said vulcanized material by applying a halogen to the shellac layer and thereafter neutralizing the indurated surface.

2. A leather substitute very closely resembling genuine dressed leather in appearance, feel, pliability, wear, durability and draping qualities, which is obtained or obtainable by coating the unnaped side of a sheeting weighing 5 ounces per square yard dyed black and having one side napped with a rubber cement of the formula

|                                                                | Per cent |
|----------------------------------------------------------------|----------|
| Plantation rubber                                              | 40       |
| Palm oil                                                       | 1        |
| Zinc oxide                                                     | 4        |
| Barytes                                                        | 25       |
| Whiting                                                        | 28       |
| Albasan (anti-oxidant)                                         | 0.4      |
| Trimene base (triethyl, trimethylene, tri-amine) (accelerator) | 1.0      |
| Sulphur                                                        | 0.5      |

until 1 to 2 ounces of cement per square yard have been deposited, applying over the said rubber cement coating a layer of a rubber composition having the formula

|                                                              | Per cent |
|--------------------------------------------------------------|----------|
| Plantation crepe                                             | 66.635   |
| Palm oil                                                     | 1.000    |
| Carbon black                                                 | 3.500    |
| Zinc oxide                                                   | 4.000    |
| Newsprint paper                                              | 21.69    |
| "Neozone D" (phenyl beta naphthylamine) (antioxidant)        | .75      |
| Trimene base (triethyl trimethylene tri-amine) (accelerator) | 1.75     |
| Sulphur                                                      | .675     |

coating the said rubber composition with a thin coat of quick drying shellac varnish, embossing the resulting laminated sheet material, vulcanizing the said embossed material, indurating the

said vulcanized material by applying a halogen to the shellac layer and thereafter neutralizing the indurated surface.

3. An artificial leather comprising a backing of fabric napped on one side and having secured to the opposite side thereof a layer of vulcanized rubber cement and an indurated layer of vulcanized rubber composition containing at least 67% of rubber and the remainder wood fiber and nonearthy material, the ratio of wood fiber to rubber being from about 3 parts of rubber by weight to 1 part of fiber, said fiber being about 1 mm. to 2 mm. in length and being uniformly disintegrated and dispersed through said composition by mastication, said composition being capable of retaining during vulcanization sharp embossing marks imparted to the unvulcanized coating, and a thin halogenated layer of shellac thereon, said coating being flexible and 20 free from rubbery feel.

4. An artificial leather comprising a backing of fabric napped on one side and having secured to the opposite side thereof a layer of vulcanized rubber cement and an indurated layer of vulcanized rubber composition containing at least 67% of rubber and the remainder wood fiber and nonearthy material, the ratio of wood fiber to rubber being from about 2 to about 5 parts of rubber by weight to 1 part of fiber, said fiber being about 1 mm. to 2 mm. in length and being uniformly disintegrated and dispersed through said composition by mastication, said composition being capable of retaining during vulcanization sharp embossing marks imparted to the unvulcanized coating, and a thin halogenated layer of shellac thereon, said coating being flexible and 35 free from rubbery feel.

5. An artificial leather comprising a backing of fabric napped on one side and having secured to the opposite side thereof a layer of vulcanized rubber cement and an indurated layer of vulcanized rubber composition containing at least 50% and not more than about 75% of rubber and the remainder wood fiber, curing ingredients including sulphur and coloring material, the ratio of wood fiber to rubber being from about 2 to

about 5 parts of rubber by weight to 1 part of fiber the amount of rubber present being about 100 times the amount of sulphur present, said fiber being about 1 mm. to 2 mm. in length and being uniformly disintegrated and dispersed through said composition by mastication, said composition being capable of retaining during vulcanization sharp embossing marks imparted to the unvulcanized coating, and a thin halogenated layer of shellac thereon, said coating being flexible and free from rubbery feel.

6. An artificial leather comprising a backing of fabric napped on one side and having secured to the opposite side thereof a layer of vulcanized rubber cement, a layer of vulcanized rubber composition containing at least 50% and not more than about 75% rubber, and the remainder fibers of newsprint paper and non-earthly material, the ratio of newsprint paper to rubber being from about 2 to about 5 parts of rubber by weight to 1 part of newsprint paper, said newsprint paper being thoroughly and uniformly disintegrated and dispersed through said coating composition by mastication until the vulcanized coating will retain sharply and distinctly embossing marks which are imparted to the unvulcanized coating before vulcanization, said coating being flexible and free from rubbery feel.

7. A coating composition suitable for coating flexible base material for the manufacture of leather substitute which comprises at least 50% to about 75% rubber, and the remainder wood fiber in the form of newsprint paper, curing ingredients and coloring material to impart color and the desired vulcanizing properties to the rubber, said fiber being present in the ratio of about 1 part of fiber to about 2 to about 5 parts of rubber and being uniformly disintegrated and dispersed through the composition by mastication, the composition being capable of retaining during vulcanization sharp embossing marks which are impressed into the unvulcanized composition, and said composition being flexible and free from rubbery feel after vulcanization.

DAVID J. SULLIVAN.